

## UNITED STATES PATENT OFFICE.

HENRY A. SMITH, OF SANTA BARBARA, CALIFORNIA.

## WALL BOARD AND PROCESS OF MAKING THE SAME.

No Drawing.

Application filed September 30, 1920. Serial No. 413,802.

*To all whom it may concern:*

Be it known that I, HENRY A. SMITH, a citizen of the United States, residing at Santa Barbara, in the county of Santa Barbara and State of California, have invented new and useful Improvements in Wall Boards and Processes of Making the Same, of which the following is a specification.

My invention relates to wall board and the process of making the same.

It is an object of this invention to construct a wall board suitable for outdoor and indoor use, which is inexpensive of manufacture, durable, and which is suitable for the application of either paint or other coatings, or plaster and the like.

My invention consists in the composition of the wall board and the process of making the same hereinafter described and claimed.

The composition is made as follows: asphaltum 15%, coarse sawdust 40%, wooden slivers of the size and shape of broken tooth picks 30%, and sand 15%. The quantities given are by volume.

The asphaltum is heated to approximately 350° F., and the sawdust and slivers are thoroughly mixed therewith. The hot asphaltum mixed with sawdust and slivers as just described is applied onto a moving table which is covered with a thin layer of sand, flaky slate preferred, to prevent the hot mixture from sticking to the table. The thickness of the layer of the hot mixture applied to the table is about two inches. Another thin layer of sand is placed on the upper surface of the hot mixture and a compression roller which reduces the thickness of the layer to about five eighths of an inch, keeping the sand and roller hot to prevent chilling and cracking, delivering the layer of asphaltum and sand from the moving table to a set of compression rollers, and passing the layer between the compression rollers and thereby reducing the thickness to about three-eighths of an inch.

In place of slivers cut straw may be used.

The sawdust and the wooden fibre or the straw serves not only as a binder but also as an absorbent of the more volatile constituents of the asphaltum, making the remainder of the asphaltum much harder. The

absorption of the volatile constituents by the wooden fibre has a tendency to preserve the same and make it impervious to moisture.

In place of the sawdust, slivers or straw a mineral fibre could be substituted, such as asbestos, although ordinarily the cost of such mineral fibre is prohibitive.

The wall board produced by my method presents a smooth surface, yet having sufficient roughness to take paint, either oil or cold water, readily, as well as a coating of cement or plaster.

It will be understood that the present invention is not concerned with the particular apparatus used in making my wall board, but only the composition and method of making the same.

Various changes may be made in the process by those skilled in the art, and the proportions of the ingredients may likewise be varied without departing from the spirit of my invention as claimed.

I claim:

1. A process of making wall board comprising heating asphaltum to approximately 350° F., mixing sawdust and slivers into the asphaltum, placing the mixed mass upon a moving table covered with a thin layer of sand, reducing the mass on the table to about two inches in thickness, applying a thin layer of sand to the upper surface of the mass, applying a compression roller which reduces the thickness of the layer to about five eighths of an inch, keeping the sand and roller hot to prevent chilling and cracking, delivering the layer of asphaltum and sand from the moving table to a set of compression rollers, and passing the layer between the compression rollers and thereby reducing the thickness to about three-eighths of an inch.

2. A process of making wall board comprising heating 15% of asphaltum to about 350° F., applying 40% of coarse sawdust and 30% of wooden slivers of the size and shape of broken toothpicks and stirring the sawdust and slivers into the asphaltum thoroughly thus producing a mass containing an excess or almost an excess of sawdust and slivers, applying a thin layer of hot sand to a moving table, applying the hot mixture to the moving table on top of the sand to form a layer about two inches

thick, applying a layer of hot sand to the top of the layer of mixture, running a hot compression roller over the layer and reducing the thickness to about five-eighths of 5 an inch, and finally running the layer between compression rollers and thereby reducing it to three-eighths of an inch thick.

3. A wall board composed of 15% asphaltum, 40% coarse sawdust, 30% wood slivers, and 15% sand, the sand being applied to the faces of the board.

In testimony whereof I have signed my name to this specification.

HENRY A. SMITH.